# EUROPEAN PATENT SPECIFICATION

(11) **EP 4 325 529 B1**
(45) Date of publication and mention of the grant of the patent: **12.02.2025**
(21) Application number: 23190721.3
(22) Date of filing: 10.08.2023
(51) Int. Cl.: H01F 1/057, H01F 41/02

(54) **SINTERED R-FE-B PERMANENT MAGNET, PREPARATION METHOD AND USE THEREOF**
GESINTERTER R-FE-B-PERMANENTMAGNET, HERSTELLUNGSVERFAHREN UND VERWENDUNG DAVON
AIMANT PERMANENT R-FE-B FRITTÉ, SON PROCÉDÉ DE PRÉPARATION ET SON UTILISATION

(30) Priority: 11.08.2022 CN 202210962847
(43) Date of publication of application: 21.02.2024
(73) Proprietor: Nantong Zhenghai Magnet Co., Ltd., 226500 Jiangsu (CN); Yantai Zhenghai Magnetic Material Co., Ltd., Yantai Shandong 264006 (CN)
(72) Inventor: Li, Wei, Jiangsu, 226500 (CN); An, Zhongxi, Jiangsu, 226500 (CN); Su, Yunting, Jiangsu, 226500 (CN); Liu, Lei, Jiangsu, 226500 (CN); Jiang, Yunying, Jiangsu, 226500 (CN); Liu, Zhongyu, Jiangsu, 226500 (CN)
(74) Representative: Gille Hrabal Partnerschaftsgesellschaft mbB Patentanwälte

(56) References cited:
- EP-A1- 3 901 967
- EP-A1- 4 152 349
- CN-A- 113 782 330
- US-A1- 2014 065 004
- US-A1- 2021 319 935

## Description

The present application claims priority to the prior application with the patent application No. 202210962847.2 entitled "SINTERED R-FE-B PERMANENT MAGNET, PREPARATION METHOD AND USE THEREOF" and filed with the China National Intellectual Property Administration on August 11, 2022.

### TECHNICAL FIELD

The present disclosure belongs to the technical field of the preparation of rare earth permanent magnet materials, and particularly relates to a sintered R-Fe-B permanent magnet with grain boundary diffusion, a preparation method and an use thereof.

### BACKGROUND

Sintered neodymium-iron-boron, as the third generation rare earth permanent magnet material, mainly consists of elements such as rare earth PrNd, iron, boron, and the like, and is widely applied to the fields of various rare earth permanent magnet motors, intelligent consumer electronic products, medical devices, and the like due to its excellent magnetic properties and high cost performance. With the rapid development of low-carbon, environment-friendly, economical, and high-new technologies, the demand for sintered neodymium-iron-boron magnets is increasing day by day, which greatly drives the consumption of rare earth PrNd resources, such that the price of PrNd is gradually increased. La and Ce, as rare earth elements with chemical properties similar to those of PrNd and the most abundant reserves, have limited use in the field of rare earth permanent magnet materials due to their relatively low intrinsic magnetic properties. At present, how to increase the usage of La and Ce elements to reduce costs without affecting the magnetic properties has become one of the research subjects for saving rare earths.

In the prior art, there are mainly the following approaches to add La and Ce into magnets: the first approach is to add in an alloying way, that is, to add metal La and Ce raw materials during the smelting process; the second approach is to add by a double alloy method, that is, to prepare (R, LaCe)-Fe-B and R-Fe-B alloy slices (R is selected from one or more of Nd, Pr, Dy, Tb, Ho, and Gd), respectively, by smelting, and then press and sinter the alloy slices described above after mixing them in a certain ratio; the third approach is to attach a compound or alloy of La and Ce on the surface of the magnet and perform an appropriate heat treatment process to diffuse La and Ce into the interior of the magnet.

In the methods described above, the addition in an alloying way can cause La and Ce to enter main phase grains, such that the properties of the main phase grains, such as saturation magnetic polarization intensity, Curie temperature, magnetocrystalline anisotropy field, and the like, can be reduced, thereby reducing the initial properties of the magnet, and further limiting the application development of the magnet. However, adding La and Ce into the interior of the magnet by diffusion has technical defects, such as the complicated process, insufficient addition amounts of La and Ce, difficulty in increasing the coercivity of the magnet, and the like, so the cost performance is low, which is not conducive to the application development of the magnet. The addition of the double alloy can prevent La and Ce from entering the main phase grains to some extent, and thus, the method has gradually become a mainstream preparation process of neodymium-iron-boron magnets containing La and Ce.

However, in order to achieve the preparation of high-performance neodymium-iron-boron magnets containing La and Ce and to compensate for the reduction of magnetic properties caused by the addition of La and Ce, a certain amount of heavy rare earth elements such as Dy and Tb are usually added to improve the magnetic properties of the magnets when the La-and Ce-rich magnets are prepared, and the heavy rare earth grain boundary diffusion technology is the most effective and easily-achieved method at present. Therefore, it has been studied that the NdCeFeB double alloy and the grain boundary diffusion technology are superimposed to prepare a magnet with a high coercivity, but the properties of the obtained magnet are not as expected, which is mainly attributed to the fact that the grain boundary phase component and the grain boundary structure of the base magnet for diffusion in the heavy rare earth grain boundary diffusion technology play a decisive role in permeation of the heavy rare earth and flow dispersion of the heavy rare earth in the interior of the magnet.

In the neodymium-cerium-iron-boron magnet prepared by the double alloy method, due to the difference in the component of main and auxiliary phases, there is a significant concentration difference of the constituent elements, which seriously affects the permeation of heavy rare earth elements into the interior of the magnet, and finally, the coercivity of the magnet is not significantly improved. Due to the heterogeneity of the distribution of rare earth elements in two main phases, the grain boundary diffusion of the heavy rare earth involves a plurality of situations. In one aspect, Nd in the main phase of Nd2Fe14B is replaced by diffusion, and in another aspect, Ce in the main phase of Ce2Fe14B is replaced by diffusion. The two processes compete with each other, and the replaced Nd or Ce will further undergo a replacement process by diffusion, resulting in the replacement of the heavy rare earth into the main phase, such that the utilization rate of the heavy rare earth is not high, and the coercivity of the magnet after diffusion is poor.

US2014/065004A1 discloses a low-cost double-main-phase Ce permanent magnet alloy and its preparation method. The Ce permanent magnet alloy has a chemical formula of (Ceₓ,Re₁₋ₓ)ₐFe_{100-a-b-c}B_{b}TM_{c} in mass percent, wherein 0.4≤x≤0.8, 29≤a ≤33, 0.8≤b≤1.5, 0.5≤c≤2, Re is one or more selected from Nd, Pr, Dy, Tb and Ho elements, and TM is one or more selected from Ga, Co, Cu, Nb and Al elements; the Ce permanent magnet alloy has a double-main-phase structure with a low H_{A} phase in (Ce,Re)-Fe-B and a high H_{A} phase in Nd-Fe-B. This double-main-phase Ce permanent magnet alloy prepared by using a double-main-phase alloy method can greatly lower the production cost of magnet while maintaining excellent magnetic performances. CN113782330A discloses a preparation method of a lanthanum-cerium-added neodymium-iron-boron magnet. The lanthanum or cerium added magnet prepared by this method has higher performance.

### SUMMARY

In order to solve the above technical problems, the present disclosure provides an R-Fe-B permanent magnet with a high coercivity, a preparation method and use thereof. The present disclosure provides an R-Fe-B permanent magnet, which comprises at least a grain boundary and composite main phase grains,
wherein the grain boundary comprises an RH-rich phase distributed in the form of an agglomerate within the grain boundary between the composite main phase grains, preferably at the intersection of any adjacent three or more composite main phase grains; the RH-rich phase can also be continuously distributed along the grain boundary in the form of a thin-layer stripe;
RH in the grain boundary has a content greater than that of the RH in the main phase grains, and the RH is at least one selected from heavy rare earth metals such as Dy, Tb, Ho;
the composite main phase grain has a core-shell structure, wherein the core-shell structure comprises a core structure having an R-T-B type phase structure and a shell structure on the outer layer of the core structure;
wherein the core structure comprises Ce-rich main phase grains and Ce-poor main phase grains; Ce in the Ce-rich main phase grains has a content of 1-15 wt%; Ce in the Ce-poor main phase grains has a content of 0.1-1 wt%; and
the RH-rich phase comprises at least one heavy rare earth metal RH selected from Dy, Tb, and Ho, at least one light rare earth metal RL selected from Pr and Nd, and optionally at least one metal M selected from Ga and Cu.

According to an embodiment of the present disclosure, the RH in the grain boundary preferably has a content greater than that of the RH in the shell structure.

According to an embodiment of the present disclosure, the permanent magnet comprises RL, wherein the RL is at least one selected from light rare earth metals such as Pr and Nd.

According to an embodiment of the present disclosure, RL in the shell structure has a content greater than or equal to that of the RL in the core structure.

According to an embodiment of the present disclosure, the permanent magnet has a structure as shown in FIG. 1, and the permanent magnet comprises at least: a grain boundary and composite main phase grains, wherein the composite main phase grain has a core-shell structure, wherein a core structure comprises Ce-rich main phase grains and Ce-poor main phase grains, and the outer layer of the core structure is provided with a shell structure; RL in the shell structure has a content greater than or equal to that of the RL in the core structure, and RH in the grain boundary has a content greater than that of the RH in the main phase grains.

According to an embodiment of the present disclosure, the R-T-B type phase structure comprises at least the following components:
R, with a weight percentage of 28% ≤ R ≤ 35%, wherein the R is selected from neodymium (Nd) and cerium (Ce), and optionally comprises or does not comprise at least one selected from scandium (Sc), yttrium (Y), lanthanum (La), cerium (Ce), praseodymium (Pr), samarium (Sm), europium (Eu), gadolinium (Gd), terbium (Tb), dysprosium (Dy), holmium (Ho), erbium (Er), thulium (Tm), ytterbium (Yb), and lutetium (Lu);
B, with a weight percentage of 0.8% ≤ B≤ 1.2%;
M, with a weight percentage of 0 ≤ M ≤5%, wherein the M is at least one selected from aluminum (Al), titanium (Ti), copper (Cu), gallium (Ga), zirconium (Zr), and niobium (Nb); and
the balance of T, wherein the T consists of iron (Fe) and optionally cobalt (Co).

According to an embodiment of the present disclosure, the permanent magnet, from the surface to the core, has phase structures of the grain boundary and the composite main phase grains described above. The core of the permanent magnet in the present disclosure refers to a position at least 500 µm away from the surface of the permanent magnet.

According to an embodiment of the present disclosure, the content of Ce in the grain boundary phase is not particularly limited.

The present disclosure further provides a preparation method of the permanent magnet described above, which comprises
mixing a powder of a low-Ce master alloy and a powder of a high-Ce auxiliary alloy, wherein Ce in the low-Ce master alloy has a content of 0.1-1 wt% and Ce in the high-Ce auxiliary alloy has a content greater than 1 wt% and not greater than 15 wt%,
performing a press molding on the mixed powder under the action of a magnetic field to obtain a green body,
performing a sintering treatment on the green body to obtain a blank, and
performing a composite diffusion treatment on the surface of the blank with a diffusion material to obtain the permanent magnet, wherein the diffusion material comprises RH, RL and optionally an M powder, wherein the RH is at least one heavy rare earth metals selected from Dy, Tb, and Ho; the RL is at least one light rare earth metals selected from Pr and Nd; and the M powder is selected from Ga and/or Cu.

Preferably, Ce in the low-Ce master alloy has a content not greater than 1 wt%, such as 0.1 wt%, 0.2 wt%, 0.3 wt%, 0.4 wt%, 0.5 wt%, 0.6 wt%, 0.7 wt%, 0.8 wt%, 0.9 wt%, or 1 wt%.

Preferably, Ce in the high-Ce auxiliary alloy has a content greater than 1 wt% and not greater than 15 wt%, such as 1 wt%, 2 wt%, 3 wt%, 4 wt%, 5 wt%, 6 wt%, 7 wt%, 8 wt%, 9 wt%, 10 wt%, 11 wt%, 12 wt%, 13 wt%, 14 wt%, or 15 wt%.

According to an embodiment of the present disclosure, the powder of the low-Ce master alloy and the powder of the high-Ce auxiliary alloy may be prepared by methods known in the art, such as hydrogen decrepitation, dehydrogenation, and milling of alloy slices. The hydrogen decrepitation, dehydrogenation, and milling may be performed by methods known in the art.

As an example, the low-Ce master alloy is prepared into a master alloy slice, which is then subjected to hydrogen decrepitation, dehydrogenation, and milling to obtain a powder of the low-Ce master alloy.

As an example, the high-Ce auxiliary alloy is prepared into an auxiliary alloy slice, which is then subjected to hydrogen decrepitation, dehydrogenation, and milling to obtain a powder of the high-Ce auxiliary alloy.

According to an embodiment of the present disclosure, the powder of the low-Ce master alloy and the powder of the high-Ce auxiliary alloy are in a mass ratio of (1-50):1, such as 1:1, 5:1, 10:1, or 20:1.

Preferably, the magnetic field may be a magnetic field known in the art, for example, a magnetic field with a magnetic field intensity of 2 T.

According to an embodiment of the present disclosure, the press molding may be performed using devices known in the art, for example, in the cavity of a press and grinding tool.

According to an embodiment of the present disclosure, after press molding, cold isostatic pressing treatment can also be performed to further improve the density of the blank.

According to an embodiment of the present disclosure, the sintering treatment comprises heating the green body to 1000-1100 °C under a vacuum atmosphere to obtain a blank.

According to an embodiment of the present disclosure, the composite diffusion treatment comprises: arranging the diffusion material on the surface of the blank, and performing heat treatment.

According to an embodiment of the present disclosure, the diffusion material may be arranged on the surface of the blank by methods known in the art, and the present disclosure is not particularly limited.

According to an embodiment of the present disclosure, the surface of the blank is uniformly coated with a slurry containing the diffusion material.

According to an embodiment of the present disclosure, the diffusion material comprises the following components: RH with a content of 20-70 wt%, RL with a content of 20-70 wt%, and an M powder with a content of 0-10 wt%.

Preferably, the RH, the RL, and the M powder in the diffusion material are in a mass ratio of (1-10):(1-5):(0-2), such as 8:3:0, 4:4:0, or 4:3.5:0.5.

According to an embodiment of the present disclosure, the RH and the RL are provided by powders of the RH and the RL, respectively.

Preferably, the powder of the RH is at least one selected from a single metal of the RH, an alloy of the RH, an oxide of the RH, a fluoride of the RH, a hydride of the RH, and an oxyfluoride of the RH. As an example, the powder of the RH is at least one selected from a single metal of Dy, an alloy of Dy, an oxide of Dy, a fluoride of Dy, a hydride of Dy, and an oxyfluoride of Dy. As an example, the powder of the RH is at least one selected from a single metal of Tb, an alloy of Tb, an oxide of Tb, a fluoride of Tb, a hydride of Tb, and an oxyfluoride of Tb. As an example, the powder of the RH is at least one selected from a single metal of Ho, an alloy of Ho, an oxide of Ho, a fluoride of Ho, a hydride of Ho, and an oxyfluoride of Ho.

Preferably, the powder of the RL is at least one selected from a single metal of the RL, an alloy of the RL, an oxide of the RL, a fluoride of the RL, a hydride of the RL, and an oxyfluoride of the RL. As an example, the powder of the RL is at least one selected from a single metal of Pr, an alloy of Pr, an oxide of Pr, a fluoride of Pr, a hydride of Pr, and an oxyfluoride of Pr. As an example, the powder of the RL is at least one selected from a single metal of Nd, an alloy of Nd, an oxide of Nd, a fluoride of Nd, a hydride of Nd, and an oxyfluoride of Nd.

According to an embodiment of the present disclosure, a diffusion adjuvant and/or a solvent may also be added to the diffusion material, wherein the diffusion adjuvant and the solvent are selected from materials known in the art, for example, the diffusion adjuvant is 4-hexylresorcinol and the solvent is ethanol.

Preferably, the amount of the diffusion adjuvant and/or the solvent used in the present disclosure is not particularly limited as long as the diffusion of the diffusion material described above can be achieved.

As an example, the RH, the diffusion adjuvant, and the solvent in the diffusion material are in a mass ratio of (1-5):(0-3):(0-3), such as 4:2:1.

In the present disclosure, due to the significant difference in the component of the composite main phase grains and the interior of the single composite main phase grain, the chemical components and the heterogeneity of the distribution cause the interior of the permanent magnet to have short-range strong exchange effect and long-range magnetostatic coupling effect, thereby effectively improving the nucleation fields of reversal magnetization domain nuclei of the permanent magnet, inhibiting the nucleation of the reversal magnetization domain nuclei, hindering the expansion of the reversal magnetization domain nuclei, and further significantly improving the coercivity of the permanent magnet.

However, when a permanent magnet is prepared by a single alloy process using Ce or Nd and a composite diffusion process, or a permanent magnet is prepared by a double alloy process using Nd and Ce and an RH diffusion process, the same performance level cannot be achieved, because the components of main phase grains are substantially equivalent and are homogeneous, and a long-range magnetostatic coupling effect cannot be formed, such that the Hcj performance equivalent to that of the present disclosure cannot be obtained under the same components and process conditions.

The present disclosure further provides use of the permanent magnet described above, such as in a motor.

### Advantageous Effects

1. The permanent magnet prepared in the present disclosure comprises two different composite main phase grains, and the long-range magnetostatic coupling effect between the grains and the short-range strong exchange effect inside the single composite main phase grain enable the permanent magnet to have a high coercivity magnetic property.
2. By means of a composite diffusion treatment, the present disclosure can ensure that heavy rare earth elements arranged on the surface of the permanent magnet diffuse more deeply and have better diffusion effect, and the core of the permanent magnet far away from the surface (that is, a position 500 µm away from the surface) also has the composite phase structural characteristics described above, such that the organization of the whole permanent magnet presents distribution uniformity, thereby effectively improving the coercivity and the squareness of the permanent magnet, and significantly improving the capacity of resisting demagnetization of the permanent magnet at a high temperature.
3. In addition, by means of composite diffusion sources, the present disclosure effectively reduces the melting point of a grain boundary phase, increases the diffusion channel of the heavy rare earth elements, improves the diffusion distance of the heavy rare earth elements in the permanent magnet, ensures that each microscopic region in the permanent magnet can form composite main phase grains, and improves the distribution uniformity of the organization structure, thereby further improving the Hcj and the squareness of the permanent magnet.

### BRIEF DESCRIPTION OF THE DRAWINGS

FIG. 1 is a schematic diagram showing the characteristics of a main phase and a grain boundary phase of the surface layer of a permanent magnet in Example 1-1.
FIG. 2 is a scanning electron microscopic back scattering image of the core (50 µm away from the surface of the permanent magnet) of the permanent magnet in Example 1-1.
FIG. 3 is EPMA images of Dy element and Pr element on a cross section of the core (50 µm away from the surface of the permanent magnet) of the permanent magnet in Example 1-1 (a is a distribution image of the Dy element, and b is a distribution image of the Pr element).
FIG. 4 is an EPMA image in which the content of Ce element is linearly scanned through the main phase grains on the cross section of the core (50 µm away from the surface of the permanent magnet) of the permanent magnet in Example 1-1.
FIG. 5 is a scanning electron microscopic back scattering image of the core (50 µm away from the surface of the permanent magnet) of the permanent magnet (a) and an EMPA image of the Dy element on the cross section of the core (b) in Comparative Example 1-1.

### DETAILED DESCRIPTION

The technical solutions of the present disclosure will be further illustrated in detail with reference to the following specific examples. It will be understood that the following examples are merely exemplary illustrations and explanations of the present disclosure, and should not be construed as limiting the protection scope of the present disclosure. All techniques implemented based on the content of the present disclosure described above are included within the protection scope of the present disclosure.

Unless otherwise stated, the raw materials and reagents used in the following examples are all commercially available products or can be prepared using known methods.

### Example 1-1 (outside the scope of the invention)

The preparation method of an R-Fe-B permanent magnet was as follows:
(1) Preparation of alloy slices: according to components of a main phase alloy and an auxiliary phase alloy as shown in Table 1, raw materials were weighed out, respectively, and main phase alloy slices and auxiliary phase alloy slices were prepared in the following way: smelting in a vacuum induction smelting furnace under Ar atmosphere, and casting the molten liquid onto a quenching roller with a rotating speed of 32 rpm at a liquid casting temperature of 1400 °C to obtain the main phase alloy slices with an average thickness of 0.25 mm and the auxiliary phase alloy slices with an average thickness of 0.30 mm;
(2) Preparation of alloy powders: the main phase alloy slices and the auxiliary phase alloy slices were prepared into a main phase alloy powder and an auxiliary phase alloy powder with average grain diameters of 3.0 µm and 2.8 µm through hydrogen decrepitation, dehydrogenation, and air flow milling, respectively.
The main phase alloy powder and the auxiliary phase alloy powder were mixed in a mass ratio of 3:1 under N₂ atmosphere, an anti-oxidation lubricant accounting for 0.05 wt% was added, and the mixture was stirred and mixed uniformly;
(3) Press molding: the mixed powder was filled into a die cavity of a die of a pressing device under N₂ atmosphere, subjected to oriented-press molding with an orientation magnetic field intensity of 3 T, and then subjected to an isostatic pressing treatment in an isostatic pressing machine under a pressure of 180 MPa to obtain a pressed compact;
(4) Sintering treatment: the pressed compact in step (3) was placed in a vacuum sintering furnace, heated to 300-400 °C at a heating rate of 3 °C/min, and heated to 670 °C at a heating rate of 5 °C/min. The temperature was kept at 670 °C for 70 min, and the pressed compact was heated to 1040 °C at a heating rate of 8 °C/min and subjected to sintering treatment for 5 h. The pressed compact was then subjected to a first-stage aging treatment at 900 °C for 4 h and a second-stage aging treatment at 530 °C for 3 h to obtain a sintered blank;
the blank described above was processed into a sheet with a size of 40 × 25 mm, wherein the thickness in an orientation direction was 5 mm;
(5) Diffusion treatment: ingredients were mixed according to a mass ratio of Dy single metal, Pr single metal, 4-hexylresorcinol, and ethanol of 4:4:2:1. Then the ingredients were mechanically stirred and mixed for 2 h to obtain a diffusion slurry containing Dy and Pr; the surface of the sheet obtained in step (4) was uniformly coated with the diffusion slurry described above with a coating amount of 1% of the mass of the base magnet, and the sheet was dried at 60 °C for 5 min to obtain a sheet coated with Dy and Pr metal diffusion sources. The sheet was subjected to vacuum permeation at 740 °C for 4 h, then the vacuum permeation at 930 °C for 6 h, and finally a vacuum aging treatment at 500 °C for 4.5 h to obtain an R-Fe-B permanent magnet M1 after Dy and Pr mixed diffusion treatment.

**Table 1. Raw material table for Examples 1-1 to 1-4**

| | PrNd | Ce | Tb | Co | Al | Ti | Cu | Ga | Zr | B |
|---|---|---|---|---|---|---|---|---|---|---|
| Main phase alloy | 30 | 0 | 1 | 1 | 0.5 | 0.2 | 0.1 | 0.4 | 0.2 | 1 |
| Auxiliary phase alloy | 17 | 15 | 0 | 1 | 0.2 | 0 | 0.3 | 0 | 0 | 0.98 |

### Example 1-2 (outside the scope of the invention)

The preparation method of the permanent magnet in this example was substantially the same as that in Example 1-1, except that Pr was replaced by Nd in the diffusion slurry in step (5).

### Example 1-3 (outside the scope of the invention)

The preparation method of the permanent magnet in this example was substantially the same as that in Example 1-1, except that the diffusion slurry in step (5) further comprised Cu, and the diffusion slurry was mixed according to a mass ratio of Dy single metal, Pr single metal, Cu metal, 4-hexylresorcinol, and ethanol of 4:3.5:0.5:2:1.

### Comparative Example 1-1

The preparation method of the permanent magnet in this comparative example was substantially the same as that in Example 1-1, except that the diffusion slurry in step (5) did not comprise Pr.

The test results of the magnetic properties of the sintered blank in Example 1-1 and the permanent magnets prepared in Examples 1-1 to 1-3 and Comparative Example 1-1 are shown in Table 2.

**Table 2. Magnetic properties in Examples 1-1 to 1-3 and Comparative Example 1-1**

| | Diffusion material | Hcj | Br | Squareness |
|---|---|---|---|---|
| Sintered blank | / | 1275 | 1.353 | 0.985 |
| Example 1-1 | Dy-Pr | 1795 | 1.334 | 0.971 |
| Example 1-2 | Dy-Nd | 1805 | 1.337 | 0.973 |
| Example 1-3 | Dy-Pr-Cu | 1810 | 1.332 | 0.977 |
| Comparative Example 1-1 | Dy | 1671 | 1.341 | 0.951 |

FIG. 1 is a schematic diagram showing the characteristics of a main phase and a grain boundary phase of the surface layer of the permanent magnet in Example 1-1.

FIG. 2 is a schematic diagram showing the characteristics of a main phase and a grain boundary phase of the core (500 µm away from the surface of permanent magnet) of the permanent magnet in Example 1-1.

FIG. 3 is EPMA images of Dy element and Pr element on a cross section of the core (50 µm away from the surface of the permanent magnet) of the permanent magnet in Example 1-1 (the left image is a distribution image of the Dy element, and the right image is a distribution image of the Pr element).

FIG. 4 is an EPMA image in which the content of Ce element is linearly scanned through the main phase grains on the cross section of the core (50 µm away from the surface of the permanent magnet) of the permanent magnet in Example 1-1.

As can be seen from FIGs. 1 to 4, the permanent magnet comprises at least a grain boundary and composite main phase grains, wherein the grain boundary comprises an RH-rich phase distributed in the form of an agglomerate within the grain boundary between the composite main phase grains, preferably at the intersection of any adjacent three or more composite main phase grains, and the RH-rich phase is continuously distributed along the grain boundary in the form of a thin-layer stripe.

As can be seen from FIGs. 2 and 3, the RH-rich phase in the permanent magnet is a bright white region in the back scattering imaging mode of the scanning electron microscope, and is distributed between adjacent main phase grains or at the intersection of three or more main phase grains, and the content of the RH in the RH-rich phase is greater than that of the RH in the main phase grains.

As can be seen from FIGs. 2 and 4, the composite main phase grains include Ce-rich main phase grains and Ce-poor main phase grains, which are dark gray regions in the back scattering imaging mode of the scanning electron microscope; in the Ce-rich main phase grains, the content of Ce is 14.5 wt%; in the Ce-poor main phase grains, the content of Ce is 0.5 wt%.

As can be seen from FIGs. 2 and 3, the composite main phase grain has a core-shell structure, wherein the shell structure is a light gray region in the back scattering imaging mode of the scanning electron microscope, which is enriched with RL elements, and the content of the RL in the shell structure is greater than or equal to that of the RL in the core structure.

Further, FIG. 3 is a distribution image of the Dy element on the cross section of the core (50 µm away from the surface of the permanent magnet) of the permanent magnet in Example 1-1, and FIG. 5 is a distribution image of the Dy element on the cross section of the core (50 µm away from the surface of the permanent magnet) of the permanent magnet in Comparative Example 1-1. As can be seen from FIGs. 3 and 5, the sintered blanks with the same component in Example 1-1 and Comparative Example 1-1 were used for composite diffusion treatment. As can be seen from the measurement results in FIGs. 3 and 4, the change in the diffusion treatment method did not cause a change in the Dy content in the interior of the magnet along the diffusion direction, but the coercivity in the interior of the magnet was greatly improved. The inventors believed that the difference in the coercivity of the permanent magnets obtained by the two diffusion methods was not caused by the concentration gradient, but by the difference in microstructure. As can be seen by observing the cross section at the position 50 µm away from the surface of the permanent magnet, the Dy element in the sample of Example 1 formed more continuous enriched streaks along the grain boundary, whereas the Dy element in the sample of Comparative Example 1 was not enriched at the grain boundary but was replaced into the main phase by a diffusion replacement process. This is because when RL is contained in the diffusion material, it diffuses into the main phase more easily than RH, causing the main phase to form a core-shell structure. The content of the RL in the shell structure of the surface of the permanent magnet is relatively high, such that the RH in the diffusion material can be prevented from being replaced into the main phase structure, and thus the Dy element can diffuse along the grain boundary to the core of the permanent magnet.

According to the above analysis, the RH element in the grain boundary phase of the permanent magnet prepared by the present disclosure can diffuse into the deeper position of the core away from the surface layer of the permanent magnet, indicating that the composite diffusion treatment effect of the present disclosure is good.

### Example 2-1

The preparation method of the permanent magnet in this example was substantially the same as that in Example 1-1, except that the raw materials were weighed out according to components of a main phase alloy and an auxiliary phase alloy as shown in Table 3, respectively.

**Table 3. Raw material table for Examples 2-1 to 2-3 and Comparative Example 2-1**

| | PrNd | Ce | Tb | Co | Al | Ti | Cu | Ga | Zr | B |
|---|---|---|---|---|---|---|---|---|---|---|
| Main phase alloy | 30 | 1 | 1 | 1 | 0.5 | 0.2 | 0.1 | 0.4 | 0.2 | 1 |
| Auxiliary phase alloy | 17 | 15 | 0 | 1 | 0.2 | 0 | 0.3 | 0.0 | 0 | 0.98 |

### Example 2-2

The preparation method of the permanent magnet in this example was substantially the same as that in Example 2-1, except that Pr was replaced by Nd in the diffusion slurry in step (5).

### Example 2-3

The preparation method of the permanent magnet in this example was substantially the same as that in Example 2-1, except that the diffusion slurry in step (5) further comprised Cu, and the diffusion slurry was mixed according to a mass ratio of Dy single metal, Pr single metal, Cu metal, 4-hexylresorcinol, and ethanol of 4:3.5:0.5:2:1.

### Comparative Example 2-1

The preparation method of the permanent magnet in this comparative example was substantially the same as that in Example 2-1, except that the diffusion slurry in step (5) did not comprise Pr.

The test results of the magnetic properties of the sintered blank in Example 2-1 and the permanent magnets prepared in Examples 2-1 to 2-3 and Comparative Example 2-1 are shown in Table 4.

**Table 4. Magnetic properties in Examples 2-1 to 2-3 and Comparative Example 2-1**

| | Diffusion material | Hcj | Br | Squareness |
|---|---|---|---|---|
| Sintered blank | / | 1215 | 1.344 | 0.986 |
| Example 2-1 | Dy-Pr | 1720 | 1.315 | 0.970 |
| Example 2-2 | Dy-Nd | 1730 | 1.311 | 0.974 |
| Example 2-3 | Dy-Pr-Cu | 1732 | 1.313 | 0.978 |
| Comparative Example 2-1 | Dy | 1628 | 1.321 | 0.953 |

As can be seen from Tables 3 and 4, the Hcj of the permanent magnet increased significantly when the composite diffusion material comprised RH and RL.

### Comparative Example 3

The preparation method of the permanent magnet in this comparative example was substantially the same as that in Example 1-1, except that the raw materials were weighed out according to components of a main phase alloy and an auxiliary phase alloy as shown in Table 5, respectively.

**Table 5. Raw material table for Comparative Example 3**

| | PrNd | Ce | Tb | Co | Al | Ti | Cu | Ga | Zr | B |
|---|---|---|---|---|---|---|---|---|---|---|
| Main phase alloy | 30 | 1.5 | 1 | 1 | 0.5 | 0.2 | 0.1 | 0.4 | 0.2 | 1 |
| Auxiliary phase alloy | 17 | 15 | 0 | 1 | 0.2 | 0 | 0.3 | 0.0 | 0 | 0.98 |

The test results of the magnetic properties of the sintered blank and the permanent magnet prepared in Comparative Example 3 are shown in Table 6.

**Table 6. Magnetic properties in Comparative Example 3**

| | Diffusion material | Hcj | Br | Squareness |
|---|---|---|---|---|
| Sintered blank | | 1201 | 1.339 | 0.985 |
| Comparative Example 1 | Dy-Pr | 1589 | 1.312 | 0.947 |

As can be seen by comparing Tables 2, 4, and 6, when Ce in the main phase alloy was 0-1% and the composite diffusion treatment was performed, the properties were significantly improved, whereas when the main phase alloy was not in the range, the improvement of the coercivity of the sintered blank was limited.

### Comparative Example 4

The preparation method of the permanent magnet in this comparative example was substantially the same as that in Example 1-1, except that an alloy was prepared by weighing the raw materials as shown in Table 7, that is, a blank was not prepared using a main phase alloy and an auxiliary phase alloy.

**Table 7. Raw material table for Comparative Example 4**

| | PrNd | Ce | Tb | Co | Al | Ti | Cu | Ga | Zr | B |
|---|---|---|---|---|---|---|---|---|---|---|
| Alloy component | 28 | 3.75 | 0.75 | 1 | 0.43 | 0.15 | 0.15 | 0.3 | 0.15 | 1 |

The test results of the magnetic properties of the sintered blank and the permanent magnet prepared in Comparative Example 4 are shown in Table 8.

**Table 8. Magnetic properties in Comparative Example 4**

| | Diffusion material | Hcj | Br | Squareness |
|---|---|---|---|---|
| Sintered blank | | 1005 | 1.338 | 0.988 |
| Comparative Example 4 | Dy-Pr | 1221 | 1.313 | 0.941 |

The permanent magnet containing Ce was prepared by a conventional method in Comparative Example 4, that is, the raw material of Ce was added directly during smelting without using a main phase alloy and an auxiliary phase alloy to prepare a blank. As can be seen from Table 8, even if the sintered blank prepared by the conventional method was subjected to the composite diffusion treatment in the present disclosure, the improvement of the coercivity of the permanent magnet was limited. The inventors found that due to the significant difference in the component of the composite main phase grains and the interior of the single composite main phase grain, the chemical components and the heterogeneity of the distribution cause the interior of the permanent magnet to have short-range strong exchange effect and long-range magnetostatic coupling effect, thereby effectively improving the nucleation fields of reversal magnetization domain nuclei of the permanent magnet, inhibiting the nucleation of the reversal magnetization domain nuclei, hindering the expansion of the reversal magnetization domain nuclei, and further significantly improving the coercivity of the permanent magnet.

However, when a permanent magnet is prepared by a single alloy process using Ce or Nd and a composite diffusion process, or a permanent magnet is prepared by a double alloy process using Ce and Nd and an RH diffusion process, the same performance level cannot be achieved, because the components of main phase grains are substantially equivalent and are homogeneous, and a long-range magnetostatic coupling effect cannot be formed, such that the Hcj performance equivalent to that of the present disclosure cannot be obtained under the same components and process conditions.

## Claims

1. An R-Fe-B permanent magnet, wherein the permanent magnet comprises at least a grain boundary and composite main phase grains;
the grain boundary comprises an RH-rich phase distributed in the form of an agglomerate within the grain boundary between the composite main phase grains, preferably at the intersection of any adjacent three or more composite main phase grains; the RH-rich phase is continuously distributed along the grain boundary in the form of a thin-layer stripe;
RH in the grain boundary has a content greater than that of the RH in the main phase grains, and the RH is at least one selected from heavy rare earth metals such as Dy, Tb, and Ho;
the composite main phase grain has a core-shell structure, wherein the core-shell structure comprises a core structure having an R-T-B type phase structure and a shell structure on the outer layer of the core structure;
**characterized in that** the core structure comprises Ce-rich main phase grains and Ce-poor main phase grains; wherein Ce in the Ce-rich main phase grains has a content of 1-15 wt%, and Ce in the Ce-poor main phase grains has a content of 0.1-1 wt%; and the
RH-rich phase comprises at least one heavy rare earth metal RH selected from Dy, Tb, and Ho, at least one light rare earth metal RL selected from Pr and Nd, and optionally at least one metal M selected from Ga and Cu.

2. The R-Fe-B permanent magnet according to claim 1, wherein the RH in the grain boundary has a content greater than that of the RH in the shell structure;
preferably, the permanent magnet comprises RL, wherein the RL is at least one selected from light rare earth metals such as Pr and Nd;
and preferably, RL in the shell structure has a content greater than or equal to that of the RL in the core structure.

3. The R-Fe-B permanent magnet according to claim 1 or 2, wherein the R-T-B type phase structure comprises at least the following components:
R, with a weight percentage of 28% ≤ R ≤ 35%, wherein the R is selected from neodymium (Nd) and cerium (Ce), and optionally comprises or does not comprise at least one selected from scandium (Sc), yttrium (Y), lanthanum (La), cerium (Ce), praseodymium (Pr), samarium (Sm), europium (Eu), gadolinium (Gd), terbium (Tb), dysprosium (Dy), holmium (Ho), erbium (Er), thulium (Tm), ytterbium (Yb), and lutetium (Lu);
B, with a weight percentage of 0.8% ≤ B≤ 1.2%;
M, with a weight percentage of 0 ≤ M ≤5%, wherein the M is at least one selected from aluminum (Al), titanium (Ti), copper (Cu), gallium (Ga), zirconium (Zr), and niobium (Nb); and
the balance of T, wherein the T consists of iron (Fe)and optionally cobalt (Co).

4. The R-Fe-B permanent magnet according to any one of claims 1-3, wherein the permanent magnet, from the surface to the core, has phase structures of the grain boundary and the composite main phase grains.

5. A preparation method of the permanent magnet according to any one of claims 1-4, wherein the preparation method comprises
mixing a powder of a low-Ce master alloy and a powder of a high-Ce auxiliary alloy, wherein Ce in the low-Ce master alloy has a content of 0.1-1
wt% and Ce in the high-Ce auxiliary alloy has a content greater than 1 wt% and not greater than 15 wt%,
performing press molding on the mixed powder under the action of a magnetic field to obtain a green body,
performing sintering treatment on the green body to obtain a blank, and
performing a composite diffusion treatment on the surface of the blank with a diffusion material to obtain the permanent magnet, wherein the diffusion material comprises RH, RL and optionally an M powder, wherein the RH is at least one heavy rare earth metals selected from Dy, Tb, and Ho; the RL is at least one light rare earth metals selected from Pr and Nd; and the M powder is selected from Ga and/or Cu.

6. The preparation method according to claim 5, wherein the powder of the low-Ce master alloy and the powder of the high-Ce auxiliary alloy are in a mass ratio of (1-50):1.

7. The preparation method according to claim 5 or 6, wherein after the press molding, performing a cold isostatic pressing treatment to further improve the density of the blank;
preferably, the sintering treatment comprises heating the green body to 1000-1100 °C under a vacuum atmosphere to obtain a blank.

8. The preparation method according to any one of claims 5-7, wherein the composite diffusion treatment comprises: arranging the diffusion material on the surface of the blank, and performing a heat treatment;
preferably, the surface of the blank is uniformly coated with a slurry containing the diffusion material

9. The preparation method according to any one of claims 5-8, wherein the diffusion material comprises the following components: RH with a content of 20-70 wt%, RL with a content of 20-70 wt%, and an M powder with a content of 0-10 wt%;
preferably, the RH, the RL, and the M powder in the diffusion material are in a mass ratio of (1-10):(1-5):(0-2);
preferably, the RH and the RL are provided by powders of the RH and the RL, respectively;
preferably, the powder of the RH is at least one selected from a single metal of the RH, an alloy of the RH, an oxide of the RH, a fluoride of the RH, a hydride of the RH, and an oxyfluoride of the RH;
and preferably, the powder of the RL is at least one selected from a single metal of the RL, an alloy of the RL, an oxide of the RL, a fluoride of the RL, a hydride of the RL, and an oxyfluoride of the RL.

10. Use of the permanent magnet according to any one of claims 1-4, **characterized in that** the permanent magnet is used for a motor.

## Patentansprüche

1. R-Fe-B-Permanentmagnet, wobei der Permanentmagnet mindestens eine Korngrenze und zusammengesetzte Hauptphasenkörner umfasst,
wobei die Korngrenze eine RH-reiche Phase umfasst, die in Form eines Agglomerats innerhalb der Korngrenze zwischen den zusammengesetzten Hauptphasenkörnern verteilt ist, vorzugsweise an der Schnittstelle von drei oder mehr beliebigen benachbarten zusammengesetzten Hauptphasenkörnern; wobei die RH-reiche Phase in Form eines Dünnschichtstreifens kontinuierlich entlang der Korngrenze verteilt ist;
wobei RH in der Korngrenze einen Gehalt aufweist, der größer als der des RH in den Hauptphasenkörnern ist, und das RH mindestens eines ausgewählt aus schweren Seltenerdmetallen wie Dy, Tb und Ho ist;
wobei das zusammengesetzte Hauptphasenkorn eine Kern-Schale-Struktur aufweist, wobei die Kern-Schale-Struktur eine Kernstruktur mit einer Phasenstruktur vom R-T-B-Typ und eine Schalenstruktur auf der äußeren Schicht der Kernstruktur umfasst,
**dadurch gekennzeichnet, dass** die Kernstruktur Ce-reiche Hauptphasenkörner und Cearme Hauptphasenkörner umfasst, wobei Ce in den Ce-reichen Hauptphasenkörnern einen Gehalt von 1-15 Gew.-% aufweist, und Ce in den Ce-armen Hauptphasenkörnern einen Gehalt von 0,1-1 Gew.-% aufweist; und die RH-reiche Phase mindestens ein schweres Seltenerdmetall RH, ausgewählt aus Dy, Tb und Ho, mindestens ein leichtes Seltenerdmetall RL, ausgewählt aus Pr und Nd, und optional mindestens ein Metall M, ausgewählt aus Ga und Cu umfasst.

2. R-Fe-B-Permanentmagnet nach Anspruch 1, wobei das RH in der Korngrenze einen Gehalt aufweist, der größer als der des RH in der Schalenstruktur ist;
wobei der Permanentmagnet vorzugsweise RL umfasst, wobei das RL mindestens eines ausgewählt aus leichten Seltenerdmetallen wie Pr und Nd ist;
und wobei das RL in der Schalenstruktur vorzugsweise einen Gehalt größer als oder gleich dem des RL in der Kernstruktur aufweist.

3. R-Fe-B-Permanentmagnet nach Anspruch 1 oder 2, wobei die Phasenstruktur vom R-T-B-Typ mindestens die folgenden Komponenten umfasst:
R, mit einem Gewichtsprozentsatz von 28 % ≤ R ≤ 35 %, wobei das R aus Neodym (Nd) und Cer (Ce) ausgewählt ist und wahlweise mindestens eines ausgewählt aus Scandium (Sc), Yttrium (Y), Lanthan (La), Cer (Ce), Praseodym (Pr), Samarium (Sm), Europium (Eu), Gadolinium (Gd), Terbium (Tb), Dysprosium (Dy), Holmium (Ho), Erbium (Er), Thulium (Tm), Ytterbium (Yb) und Lutetium (Lu) umfasst oder nicht umfasst;
B, mit einem Gewichtsprozentsatz von 0,8 % ≤ B ≤ 1,2 %;
M, mit einem Gewichtsprozentsatz von 0 ≤ M ≤ 5 %, wobei das M mindestens eines ausgewählt aus Aluminium (Al), Titan (Ti), Kupfer (Cu), Gallium (Ga), Zirkonium (Zr) und Niob (Nb) ist; und
den Rest T, wobei das T aus Eisen (Fe) und wahlweise Kobalt (Co) besteht.

4. R-Fe-B-Permanentmagnet nach einem der Ansprüche 1-3, wobei der Permanentmagnet von der Oberfläche bis zum Kern Phasenstrukturen der Korngrenze und der zusammengesetzten Hauptphasenkörner aufweist.

5. Herstellungsverfahren für den Permanentmagneten nach einem der Ansprüche 1-4, wobei das Herstellungsverfahren umfasst
Mischen eines Pulvers aus einer Ce-armen Vorlegierung und eines Pulvers aus einer Ce-reichen Hilfslegierung, wobei Ce in der Ce-armen Vorlegierung einen Gehalt von 0,1-1 Gew.-% und Ce in der Ce-reichen Hilfslegierung einen Gehalt von mehr als 1 Gew.-% und nicht mehr als 15 Gew.-% aufweist,
Durchführen von Pressformen an dem gemischten Pulver unter Einwirkung eines Magnetfelds, um einen Grünkörper zu erhalten,
Durchführen von Sinterbehandlung an dem Grünkörper, um einen Rohling zu erhalten, und
Durchführen einer zusammengesetzten Diffusionsbehandlung auf der Oberfläche des Rohlings mit einem Diffusionsmaterial, um den Permanentmagneten zu erhalten, wobei das Diffusionsmaterial RH, RL und wahlweise ein M-Pulver umfasst, wobei das RH mindestens ein schweres Seltenerdmetall, ausgewählt aus Dy, Tb und Ho ist; das RL mindestens ein leichtes Seltenerdmetall, ausgewählt aus Pr und Nd ist; und das M-Pulver aus Ga und/oder Cu ausgewählt ist.

6. Herstellungsverfahren nach Anspruch 5, wobei das Pulver der Ce-armen Vorlegierung und das Pulver der Ce-reichen Hilfslegierung in einem Massenverhältnis von (1-50):1 vorliegen.

7. Herstellungsverfahren nach Anspruch 5 oder 6, wobei nach dem Pressformen, Durchführen einer kaltisostatischen Pressbehandlung, um die Dichte des Rohlings weiter zu verbessern;
wobei die Sinterbehandlung vorzugsweise Erwärmen des Grünkörpers auf 1000-1100 °C unter einer Vakuumatmosphäre umfasst, um einen Rohling zu erhalten.

8. Herstellungsverfahren nach einem der Ansprüche 5-7, wobei die zusammengesetzte Diffusionsbehandlung umfasst: Anordnen des Diffusionsmaterials auf der Oberfläche des Rohlings und Durchführen einer Wärmebehandlung;
wobei die Oberfläche des Rohlings vorzugsweise gleichmäßig mit einer Aufschlämmung beschichtet wird, die das Diffusionsmaterial enthält.

9. Herstellungsverfahren nach einem der Ansprüche 5-8, wobei das Diffusionsmaterial die folgenden Komponenten umfasst: RH mit einem Gehalt von 20-70 Gew.-%, RL mit einem Gehalt von 20-70 Gew.-% und ein M-Pulver mit einem Gehalt von 0-10 Gew.-%;
wobei das RH, das RL und das M-Pulver in dem Diffusionsmaterial vorzugsweise in einem Massenverhältnis von (1-10):(1-5):(0-2) vorliegen;
wobei das RH und das RL vorzugsweise jeweils durch Pulver des RH und des RL bereitgestellt werden;
wobei das Pulver des RH vorzugsweise mindestens eines ausgewählt aus einem einzelnen Metall des RH, einer Legierung des RH, einem Oxid des RH, einem Fluorid des RH, einem Hydrid des RH und einem Oxyfluorid des RH ist;
und wobei das Pulver des RL vorzugsweise mindestens eines ausgewählt aus einem einzelnen Metall des RL, einer Legierung des RL, einem Oxid des RL, einem Fluorid des RL, einem Hydrid des RL und einem Oxyfluorid des RL ist.

10. Verwendung des Permanentmagneten nach einem der Ansprüche 1-4, **dadurch gekennzeichnet, dass** der Permanentmagnet für einen Motor verwendet wird.

## Revendications

1. Aimant permanent R-Fe-B, dans lequel l''aimant permanent comprend au moins un joint de grain et des grains de phase principale composites ;
le joint de grain comprend une phase riche en RH répartie sous la forme d'un agglomérat au sein du joint de grain entre les grains de phase principale composites, de préférence à l'intersection de trois quelconques grains adjacents ou plus parmi les grains de phase principale composites ; la phase riche en RH est répartie en continu le long du joint de grain sous la forme d'une bande de couche mince ;
RH dans le joint de grain a une teneur supérieure à celle du RH dans les grains de phase principale, et le RH est au moins l'un choisi parmi des métaux terreux rares lourds tels que Dy, Tb et Ho ;
le grain de phase principale composite a une structure noyau-enveloppe, dans lequel la structure noyau-enveloppe comprend une structure noyau ayant une structure de phase de type R-T-B et une structure d'enveloppe sur la couche extérieure de la structure noyau ;
**caractérisé en ce que** la structure noyau comprend des grains de phase principale riches en Ce et des grains de phase principale pauvres en Ce ; dans lequel Ce dans les grains de phase principale riches en Ce a une teneur de 1 à 15 % en poids, et Ce dans les grains de phase principale pauvres en Ce a une teneur de 0,1 à 1 % en poids ; et la phase riche en RH comprend au moins un métal terreux rare lourd RH choisi parmi Dy, Tb et Ho, au moins un métal terreux rare léger RL choisi parmi Pr et Nd, et facultativement au moins un métal M choisi parmi Ga et Cu.

2. Aimant permanent R-Fe-B selon la revendication 1, dans lequel le RH dans le joint de grain a une teneur supérieure à celle du RH dans la structure d'enveloppe ;
de préférence, l'aimant permanent comprend RL, dans lequel le RL est au moins l'un choisi parmi des métaux terreux rares légers tels que Pr et Nd ;
et de préférence, RL dans la structure d'enveloppe a une teneur supérieure ou égale à celle du RL dans la structure noyau.

3. Aimant permanent R-Fe-B selon la revendication 1 ou 2, dans lequel la structure de phase de type R-T-B comprend au moins les composants suivants :
R, avec un pourcentage en poids de 28 % ≤ R ≤ 35 %, dans lequel le R est choisi parmi néodyme (Nd) et cérium (Ce), et facultativement comprend ou ne comprend pas au moins l'un choisi parmi scandium (Sc), yttrium (Y), lanthane (La), cérium (Ce), praséodyme (Pr), samarium (Sm), europium (Eu), gadolinium (Gd), terbium (Tb), dysprosium (Dy), holmium (Ho), erbium (Er), thulium (Tm), ytterbium (Yb) et lutécium (Lu) ;
B, avec un pourcentage en poids de 0,8 % ≤ B ≤ 1,2 % ;
M, avec un pourcentage en poids de 0 ≤ M ≤ 5 %, dans lequel le M est au moins l'un choisi parmi aluminium (Al), titane (Ti), cuivre (Cu), gallium (Ga), zirconium (Zr) et niobium (Nb) ; et
le reste étant T, dans lequel le T est constitué de fer (Fe) et facultativement de cobalt (Co).

4. Aimant permanent R-Fe-B selon l'une quelconque des revendications 1 à 3, dans lequel l'aimant permanent, depuis la surface jusqu'au noyau, présente des structures de phase du joint de grain et des grains de phase principale composites.

5. Procédé de préparation de l'aimant permanent selon l'une quelconque des revendications 1 à 4, dans lequel le procédé de préparation comprend
le mélange d'une poudre d'un alliage mère à faible teneur en Ce et d'une poudre d'un alliage auxiliaire à haute teneur en Ce, dans lequel Ce dans l'alliage mère à faible teneur en Ce a une teneur de 0,1 à 1 % en poids et Ce dans l'alliage auxiliaire à haute teneur en Ce a une teneur supérieure à 1 % en poids et non supérieure à 15 % en poids,
la réalisation d'un moulage par compression sur la poudre mélangée sous l'action d'un champ magnétique pour obtenir un corps cru,
la réalisation d'un traitement par frittage sur le corps cru pour obtenir une ébauche, et
la réalisation d'un traitement par diffusion composite sur la surface de l'ébauche avec un matériau de diffusion pour obtenir l'aimant permanent, dans lequel le matériau de diffusion comprend RH, RL et facultativement une poudre M, dans lequel le RH est au moins un des métaux terreux rares lourds choisis parmi Dy, Tb et Ho ; le RL est au moins un des métaux terreux rares légers choisis parmi Pr et Nd ; et la poudre M est choisie parmi Ga et/ou Cu.

6. Procédé de préparation selon la revendication 5, dans lequel la poudre de l'alliage mère à faible teneur en Ce et la poudre de l'alliage auxiliaire à haute teneur en Ce sont dans un rapport de masse de (1-50): 1.

7. Procédé de préparation selon la revendication 5 ou 6, dans lequel après le moulage par compression, on réalise un traitement par compression isostatique à froid pour améliorer encore la masse volumique de l'ébauche ;
de préférence, le traitement par frittage comprend le chauffage du corps cru à 1000-1100 °C dans une atmosphère sous vide pour obtenir une ébauche.

8. Procédé de préparation selon l'une quelconque des revendications 5 à 7, dans lequel le traitement par diffusion composite comprend : la disposition du matériau de diffusion sur la surface de l'ébauche, et la réalisation d'un traitement thermique ;
de préférence, la surface de l'ébauche est uniformément revêtue d'une suspension épaisse contenant le matériau de diffusion

9. Procédé de préparation selon l'une quelconque des revendications 5 à 8, dans lequel le matériau de diffusion comprend les composants suivants : RH avec une teneur de 20 à 70 % en poids, RL avec une teneur de 20 à 70 % en poids, et une poudre M avec une teneur de 0 à 10 % en poids ;
de préférence, le RH, le RL et la poudre M dans le matériau de diffusion sont dans un rapport de masse de (1-10):(1-5):(0-2) ;
de préférence, le RH et le RL sont fournis par des poudres du RH et du RL, respectivement ;
de préférence, la poudre du RH est au moins l'un choisi parmi un métal unique du RH, un alliage du RH, un oxyde du RH, un fluorure du RH, un hydrure du RH, et un oxyfluorure du RH ;
et de préférence, la poudre du RL est au moins l'un choisi parmi un métal unique du RL, un alliage du RL, un oxyde du RL, un fluorure du RL, un hydrure du RL, et un oxyfluorure du RL.

10. Utilisation de l'aimant permanent selon l'une quelconque des revendications 1 à 4, **caractérisée en ce que** l'aimant permanent est utilisé pour un moteur.
